

## 1

3,426,076

OXIDATIVELY STABLE ALKYLBIPHENYLS  
AND TERPHENYLS AS NON-SPREADING  
LUBRICANTS

Helen Mertwoy, Montgomery, and Henry Gisser, Philadelphia, Pa., assignors to the United States of America as represented by the Secretary of the Army  
No Drawing. Filed July 28, 1966, Ser. No. 568,680  
U.S. Cl. 260—612 2 Claims  
Int. Cl. C10m 3/10, 3/14

## ABSTRACT OF THE DISCLOSURE

Non-spreading lubricants and fluids which are oxidatively stable at low and high temperatures and comprising a mono or di-sec-butyl-biphenyl or terphenyl or mono or di-sec-butyl-methoxybiphenyl or methoxyterphenyl.

This invention relates to fluids and lubricants and more particularly concerns new and improved nonspreading fluids which are stable to oxidation.

Many nonspreading fluids are useful as lubricants in applications such as watch mechanisms, clocks and fuzes where a continual supply of lubricating substance cannot readily be provided and where the lubricant film is placed between components having low relative speeds such that the resistance of the lubricant to spreading governs the accuracy of the mechanism. Since the nonspreading component of such nonspreading lubricant is an important factor contributing to the performance of the lubricant, control of the nonspreading ingredient will usually lead to control of the compounded lubricant. Prior art researchers have compounded lubricants from blends containing a nonspreading ingredient comprising a diester made from an aromatic alcohol and a dibasic acid, having the general formula:



where X and R are aliphatic (straight or branch chain) groups; X having up to 4 carbon atoms, R having up to 5 carbon atoms, and M is 5 through 7. The lubricant would normally contain a suitable oxidative inhibitor, among other possible additives. Since addition of oxidation inhibitors to fluids can change the physical properties thereof e.g., freezing point, and since aromatic compounds do not respond well to antioxidants, it would be advantageous if a nonspreading fluid which is also stable to oxidation could be provided.

It is therefore an object of this invention to provide improved nonspreading lubricants.

Another object of the invention is to provide improved nonspreading lubricants which are stable to oxidation up to at least 100° C.

Other objects and features of the invention will become apparent as the invention is more fully hereinafter disclosed.

In accordance with these objects it has been discovered that a mono or di-sec-butyl-biphenyl or terphenyl or mono or di-sec-butyl-methoxybiphenyl or methoxyterphenyl will provide a nonspreading oxidatively stable fluid. The alkyl group or groups will be attached to the ring through a

5

10

20

25

30

35

50

55

65

## 2

tertiary carbon atom. Examples of structures of this type are as follows:



biphenyl



o-terphenyl



m-terphenyl

R=sec-butyl

R'=sec-butyl, hydrogen, or methoxy

R''=sec-butyl or hydrogen

Since the higher the symmetry of a substituted biphenyl or terphenyl the higher the melting point, it is important that the compounds be as unsymmetrical as possible in order to obtain liquids. For example, 4,4'-di-sec-butylbiphenyl is a liquid yet 4,4'-dibutylbiphenyl (M.P. 58.5° C.) and 4,4'-di-tert-butylbiphenyl (M.P. 128.5° C.) are solids. Therefore, substituted and unsubstituted biphenyls and terphenyls were reacted with sec-butyl chloride to form liquid sec-butyl derivatives which were unsymmetrical compounds.

In Table I below, spreading data are presented for our nonspreading oxidatively stable fluids, the data being obtained at room temperature under anhydrous conditions.

TABLE I.—SPREADING DATA

| Compound                                            | Percent spreading after— |         |
|-----------------------------------------------------|--------------------------|---------|
|                                                     | 7 days                   | 30 days |
| 4-sec-butylbiphenyl                                 | 1 <sup>1</sup>           | 0.3     |
| 4,4'-di-sec-butylbiphenyl                           | 0                        | 0.3     |
| 4-sec-butyl-4'-methoxybiphenyl                      | 0.4                      | 0.9     |
| 3,4-di-sec-butyl-4'-methoxybiphenyl                 | 0                        | 0.8     |
| 4-sec-butyl-m-terphenyl                             | 0                        | 0       |
| 4,4''-di-sec-butyl-m-terphenyl                      | 0.5                      | 1.2     |
| 4-sec-butyl-o-terphenyl                             | 1.2                      | 1.5     |
| 4,4''-di-sec-butyl-o-terphenyl                      | 0                        | 0.5     |
| 4-sec-butyl-2'-methoxy-p-terphenyl                  | 5.0                      | 20.0    |
| Bis(p-isopropylbenzyl)3-methyl adipate <sup>2</sup> | 5.0                      | 115.0   |

<sup>1</sup> Evaporated.

<sup>2</sup> Compound is a known spreading fluid and is presented for comparison purposes.

Despite the high boiling point of 4-sec-butylbiphenyl (107° C. at 0.7 mm.), it completely evaporated within about 4 days leaving no residue on the disk on which it was being tested. This compound has been found useful therefore in closed systems. While a drop of 4-sec-butyl-4'-methoxybiphenyl only spreads 0.9% after 30 days, its volume had noticeably decreased indicating that this compound (B.P. 146° C. at 0.7 mm.) was also evaporating but at a much slower rate.

Spreading of an oil was determined in the following manner: One inch diameter disks of WD 52-100 steel, hardened to Rockwell C-62, were polished successively with 0, 2/0, 3/0, and 4/0 emery paper, washed under warm tap water while being scrubbed with cotton gauze, then washed with distilled water followed by redistilled methanol. The disks were then dried by clean dry air. To

determine cleanliness, a drop of redistilled methanol was placed on the surface of each disk. Complete and uniform evaporation indicated surfaces acceptable for these tests. A drop of the oil to be tested, 1 to 2 mm. in diameter, was placed on each disk by means of platinum wire. The degree of spreading was obtained by measuring the change in diameter after 7 and 30 days, respectively, using a traveling microscope.

Our nonspreading fluid may be prepared as follows using 4-sec-butyl-4'-methoxybiphenyl and 3,4-di-sec-butyl-4'-methoxybiphenyl as examples:

p-Phenylanisole (0.25 mole, 46 gm.) was dissolved in 700 ml. of hot heptane contained in a 1000 cc. four-necked flask, fitted with a stirrer, reflux condenser, thermometer and dropping funnel. Fourteen grams of anhydrous aluminum chloride were then added. The solution was heated, and while maintaining a temperature at 75-85° C., 0.27 mole (25 gm.) 2-chlorobutane was added dropwise over a period of 2.5 hours. After addition was complete, stirring was continued for an additional 5.5 hours, the temperature being maintained at 75-85° C. The reaction mixture was poured over an equal volume of cracked ice and stirred vigorously to decompose the aluminum chloride complexes. The organic layer was washed free of acid with distilled water. The unreacted p-phenylanisole was removed by distillation using a steam condenser. The remaining mixture was distilled in a molecular pot still to separate the product from solids and tarry products. The liquid was then fractionated using a Vigreux column to yield both 4 - sec. butyl - 4' - methoxybiphenyl (B.P. 137° C. at 0.65 mm.) and 3,4 - di - sec - butyl - 4' - methoxybiphenyl (B.P. 162° at 0.75 mm.). Both compounds were then fractionated for further purification using a Vigreux column until the distillation range was less than 2° C.

In view of the above, a description of the preparation of the other compounds of our invention will not be presented herein as falling within the knowledge of a skilled organic chemist.

In the table below, some oxidation rates of our inventive nonspreading compound are presented. As can be readily observed from the table, there is very little oxygen uptake even after 100 hours.

TABLE II.—OXIDATION RATES AT 100° C.

| Compound                                | (Moles O <sub>2</sub> /mole compound/hr.)<br>X10 <sup>4</sup> |                                    |
|-----------------------------------------|---------------------------------------------------------------|------------------------------------|
|                                         | Initial rate<br>during 5-35 hr.                               | Final rate<br>during 65-100<br>hr. |
| 4-sec-butylbiphenyl.....                | 0.03                                                          | 0.03                               |
| 4,4'-di-sec-butylbiphenyl.....          | 0.13                                                          | 0.17                               |
| 4-sec-butyl-4'-methoxybiphenyl.....     | 0.00                                                          | 0.00                               |
| 3,4-di-sec-4'-methoxybiphenyl.....      | 0.12                                                          | 0.20                               |
| 4-sec-butyl-m-terphenyl.....            | 0.00                                                          | 0.00                               |
| 4,4'-di-sec-butyl-m-terphenyl.....      | 0.32                                                          | 0.21                               |
| 4-sec-butyl-o-terphenyl.....            | 0.00                                                          | 0.00                               |
| 4,4'-di-sec-butyl-o-terphenyl.....      | 0.39                                                          | 0.23                               |
| 4-sec-butyl-2'-methoxy-p-terphenyl..... | 0.00                                                          | 0.00                               |

Oxygen consumption at 100° was measured by using standard Warburg manometry. One milliliter of compound was introduced into the main compartment of the Warburg flask. Since oxygen consumption in the initial stages of autoxidation was measured, it was not necessary to use absorbents for volatiles. The flask was immersed in 100° C. oil bath and allowed to come to equilibrium during which time the system was flushed with oxygen for approximately 15 minutes. When the system was finally closed to the atmosphere excess oxygen pressure was bled off so that 0.1 to 0.5 cm. of pressure remained. Oxygen consumption was calculated as moles of oxygen per mole of compound.

We claim:

1. A nonspreading fluid oxidatively stable at elevated temperatures, said fluid being 4-sec-butyl-4'-methoxybiphenyl.
2. A nonspreading fluid oxidatively stable at elevated temperatures, said fluid being 3,4-di-sec-butyl-4'-methoxybiphenyl.

#### References Cited

#### UNITED STATES PATENTS

- |           |         |                      |         |
|-----------|---------|----------------------|---------|
| 2,161,558 | 6/1939  | Coleman et al. ----- | 260—612 |
| 2,172,391 | 9/1939  | Krase.               |         |
| 2,773,906 | 12/1956 | Emerson.             |         |

BERNARD HELFIN, Primary Examiner.

U.S. Cl. X.R.  
252—52, 59; 260—668